

# UNITED STATES PATENT OFFICE

VEZIO VENDER, OF MILAN, ITALY.

## METHOD OF MAKING HORNY NITROCELLULOSE BODIES.

946,294.

Specification of Letters Patent. Patented Jan. 11, 1910.

No Drawing.

Application filed December 8, 1906. Serial No. 346,961.

To all whom it may concern:

Be it known that I, VEZIO VENDER, chemist, a subject of the King of Italy, residing in Milan, Italy, have invented certain new and useful Improvements in Methods of Making Horny Nitrocellulose Bodies, of which the following is a specification.

This invention has for its object a method of making practically unfreezable explosives of plastic horny constitution and of great permanency, and with a low explosive temperature.

By nitrating acetins which are basic with ordinary nitrosulfuric acid for making nitroglycerin there is obtained, a very poor yield of nitroglycerin which contains little nitracetin. It has been found that the sulfuric acid of the acid mixture separates acetyl, and that on the other hand a good yield of pure nitracetin can be obtained by nitrating the basic acetin with nitric acid of more than 65%  $\text{NO}_3\text{H}$  or with nitro-sulfuric acid containing more nitric acid than sulfuric acid, and that a good yield of mixtures of nitracetin and nitro-glycerin can be obtained by nitrating acetin glycerin mixtures, if acid mixtures be employed containing as much more nitric acid than sulfuric acid as there is acetin in proportion to glycerin. With the thus obtained (not yet described) pure nitracetin some valuable properties have been discovered, and important technical progress attained; it has been found that nitracetin more particularly di-nitracetin does not freeze even at very low temperatures, and that the same is the case with its mixtures with nitroglycerin; that nitracetins are extremely nonsusceptible to heat and shock, and that it is impossible to cause it to explode or ignite by means of a hammer or by striking iron against iron, and that it is so great a solvent for gun-cotton that, even when cold, gun-cotton of 13.4% N may be gelatinized and that it possesses as great an explosive power but a lower explosion temperature than nitroglycerin. In similar manner to nitracetin the hitherto unknown nitroformins are obtained by nitrating formin, and it has been found that these nitroformins have great explosive power and can so lower the freezing point of nitroglycerin that a mixture of about 25% dinitroformin with nitroglycerin may be regarded as practically unfreezable.

55 A plastic and horny consistency is to-day

regarded as absolutely necessary in explosives and smokeless powder, but the plastic horny substances hitherto employed have the drawback of freezing at a temperature below 10° C. losing their valuable properties while being slow of ignition and very dangerous. Now this invention relates to the use of acetin, formin, nitracetin, nitroformin, for making plastic horny explosives with the object of retaining their plastic horny condition at the low temperatures which are met with in practice, in other words for making practically unfreezable explosives. The use of acetin and nitracetin is preferable if the property of dissolving nitrocellulose in a great degree is required. It is thus possible to make practically unfreezable smokeless powder having a very low explosion temperature with gun-cotton of 13.4% N, and dinitracetin, without the use of other solvents or gelatinizing substances.

Dinitroformin does not possess particular gelatinizing properties for nitrocellulose, but it has great explosive power, and it is thus very well adapted for making unfreezable explosives of great power, for instance for producing gelatin dynamite rendered unfreezable by the addition of nitroformin. The use of acetin, nitracetin, formin, nitroformin for lowering the freezing point of nitroglycerin explosives, or making unfreezable explosives without nitroglycerin, affords special technical advantages over other processes proposed for the same object; they are not volatile substances, are very permanent, do not contain chlorin and are easily made, and the property of dinitracetin of easily gelatinizing gun-cotton allows of the production of horny, smokeless, unfreezable, powder having a low explosion temperature, which is not possible with the other substances proposed, as these attack metals or are volatile or hygroscopic, or are not sufficiently gelatinizing, or produce a high explosion temperature. It has also been found that if acetin soluble in water be employed as gelatinizing substance for nitrocellulose, it is possible to employ this acetin as an aqueous solution (if afterward the water be evaporated) in order to produce the gelatinizing. And it has been found that the acetin employed may be easily washed out of the gelatinous substances obtained with acetin soluble in water, yielding horny substances of the original (that is the important) form.

This peculiar method can only be carried out with nonvolatile acetin, soluble in water, and is quite different from the methods hitherto known of using the volatile or 5 gelatinizing substances non-soluble in water, and affords valuable technical advantages, as it allows of the use of wet nitrocellulose and non-volatile, non-inflammable gelatinizing substances and of an absolutely uniform 10 distribution of the gelatinizing substances; and, then gradual action (by evaporating the water) of the gelatinizing substances, so that quite homogeneous horny substances may be obtained, as gelatinizing substances are 15 easily homogeneously diffused as aqueous solution (not emulsion); also by the use of these gelatinizing substances soluble in water, an easy removal and recovery of the gelatinizing substances (acetin) is possible even 20 if the bodies possess great density, without danger of inflammability or injury to health.

The process will now be more particularly explained in connection with the following examples:—

25 Example I: 160 kgs. of wet nitrocellulose (or 100 kgs. of dry nitrocellulose) are moistened, saturated or kneaded with a solution of 60 kgs. of acetin in 100 kgs. of water; a paste is formed, and then the water is evaporated; the remaining acetin gelatinizes the 30 nitrocellulose.

Example II: The bodies obtained by gelatinizing nitrocellulose with acetin soluble in water, for instance in the manner described 35 in the preceding example, and in a granular, thread-like or other appropriate form, are washed with warm water. The water easily removes the acetin, and horny bodies of

nitrocellulose are obtained in the original form of grains or threads.

Example III: 200 kgs. of wet nitrocellulose (100 kgs. of dry nitrocellulose) are formed by the usual methods in grains, and these are moistened or saturated with a solution of 30 kgs. of mono-acetin in 30 kgs. of 45 water. The soft wet grains are now dried and the remaining concentrated acetins gelatinize the nitrocellulose. The grains thus gelatinized are washed with warm water which removes the acetin. Horny grains of 50 nitrocellulose are obtained, making a very good smokeless powder.

I claim as my invention:

1. A method of making horny nitrocellulose bodies of determinate form which consists in gelatinizing nitrocellulose bodies of the desired form with acetin soluble in water, and subsequently treating the substances with an aqueous fluid for the purpose of removing and recovering the gelatinizing substance. 55

2. A method of making explosives of the class described consisting in incorporating an aqueous solution of acetin as a gelatinizing agent, with nitrocellulose, evaporating the water from the solution to effect a gelatinizing action, and subsequently treating the substances with an aqueous fluid for the purpose of removing and recovering the gelatinizing substance. 60 65

In testimony whereof I affix my signature 70 in presence of two witnesses.

VEZIO VENDER.

Witnesses:

B. CARLO SALVOTI,  
M. SIERSELORFER, JR.